

## UNITED STATES PATENT OFFICE.

GEORGE H. CHARLS, OF CANTON, OHIO, ASSIGNOR TO UNITED ALLOY STEEL CORPORATION, OF CANTON, OHIO, A CORPORATION OF NEW YORK.

## RESISTANT-SURFACE ALLOY OF IRON.

No Drawing.

Application filed April 14, 1924. Serial No. 706,567.

To all whom it may concern:

Be it known that I, GEORGE H. CHARLS, a citizen of the United States, and a resident of Canton, Stark County, State of 5 Ohio, have invented an Improvement in Resistant-Surface Alloys of Iron, of which the following is a specification.

This invention relates to iron alloys. One of the objects thereof is to provide a practical alloy of iron of such nature that its surface will be dependably resistant to severe corroding or discoloring influences and will maintain its original character and appearance. Another object is to provide an 15 alloy in which the above advantages are attained without sacrifice of physical properties or undue increase of cost. Other objects will be in part obvious or in part pointed out hereinafter.

20 The invention accordingly consists in the combinations of constituents and in the ideas and features herein illustratively described, and the scope of the application of which will be indicated in the appended 25 claims.

As an illustrative embodiment of this invention which I have found to give excellent results, I include the following elements in the following proportions: chromium 30 from 16.0% to 20.0%, and molybdenum from .05% to .12%. These are incorporated in an iron alloy, and it may be noted that the term "iron alloy" is broadly used to include compositions in which carbon 35 may or may not be present according as it is or is not specified.

It is also to be noted that the term "resistant-surface" is used to denote a characteristic of the metal whereby it, throughout its entire mass, is adapted to present a surface which strongly resists any tendencies to discoloration, corrosion, or other alteration by heat or any other agency.

The carbon is preferably kept low, by 45 which is meant, in this connection, .20% or under. In fact, I have found highly desirable results with a carbon range of from .03% to .07%.

Elements such as phosphorous and sulphur, usually present in all commercial iron and steel, should be kept as low as possible.

There is preferably added an amount of vanadium of around .10% to .50% to act as

a scavenger and thus permit the remaining 55 elements to coact to the best effect, and it is to be understood that this element, as well as the others above set forth, is preferably added in such manner as to diffuse uniformly throughout the mass of the metal. 60

The ranges above set forth are by no means limiting, as very considerable deviations therefrom may be made and substantial benefit of the invention retained. Accordingly, in certain of the claims, ranges 65 of the constituent elements broader than the above preferred range are specified by setting higher or lower limiting percentages. The element molybdenum, however, is preferably kept low, in fact its full effect in imparting a resistant surface to the alloy is attained below .35%, and a substantially smaller amount gives better results. 70

Alloys such as that above described will be found to achieve the objects of this 75 invention and the advantages hereinabove noted all without special heat treatment.

As variations might be made in the embodiment of my invention herein described without departure from its scope, it is to 80 be understood that all matter herein is to be interpreted as illustrative and not in a limiting sense.

I claim as my invention:

1. A resistant-surface alloy of iron containing as the principal elements, in combination with the iron, silicon from .50% to 85 6.0%, chromium from 3.0% to 30.0%, and molybdenum in an effective amount not exceeding .35%. 90

2. A resistant-surface alloy of iron containing as the principal elements, in combination with the iron, silicon from .50% to 6.0%, chromium from 3.0% to 30.0%, molybdenum in an effective amount not exceeding .35%, and carbon in an effective amount not exceeding .20%. 95

3. A resistant-surface alloy of iron containing as the principal elements, in combination with the iron, chromium from 16.0% to 25.0%, silicon from 1.0% to 4.0%, molybdenum in an effective amount not exceeding .35%, and carbon in an effective amount not exceeding .10%. 100

4. A resistant-surface alloy of iron containing as the principal elements, in combination with the iron, molybdenum from .05% to 20%, chromium from 3.0% to 105

25.0%, silicon from .50% to 5.0%, and carbon in an effective amount not exceeding .20%.

5. A resistant-surface alloy of iron containing as the principal elements, in combination with the iron, chromium from 16.0% to 25.0%, molybdenum from .05% to .20%, silicon from .50% to 5.0%, and carbon in an effective amount not exceeding .20%.

10. 6. A resistant-surface alloy of iron containing as the principal elements, in combination with the iron, silicon from 1.3% to 4.0%, chromium from 3.0% to 25.0%, and molybdenum in an effective amount not exceeding .35%.

15. 7. A resistant-surface alloy of iron containing as the principal elements, in combination with the iron, silicon from 1.3% to 4.0%, chromium from 3.0% to 25.0%, molybdenum in an effective amount not exceeding .35%, and carbon in an effective amount not exceeding .10%.

20. 8. A resistant-surface alloy of iron containing as the principal elements, in combi-

nation with the iron, molybdenum from .05% to .20%, chromium from 16.0% to 25.0%, silicon from 1.0% to 4.0%, and carbon in an effective amount not exceeding .10%.

25. 9. A resistant-surface alloy of iron containing as the principal elements, in combination with the iron, molybdenum from .05% to .12%, chromium from 16.0% to 20.0%, silicon from 1.0% to 2.50%, and carbon from .03% to .07%.

30. 10. A resistant-surface alloy of iron containing as the principal elements, in combination with the iron, chromium from 3.0% to 30.0%, silicon from .50% to 6.0%, carbon in an effective amount not exceeding .20%, 40 molybdenum in an effective amount not exceeding .35%, and vanadium in an appreciable amount not exceeding .50%.

35. In testimony whereof, I have signed my name to this specification this third day of April, 1924.

GEORGE H. CHARLS.